

# United States Patent [19]

Nagaraj

[11] Patent Number: 4,595,493

[45] Date of Patent: Jun. 17, 1986

[54] PROCESS FOR THE FLOTATION OF BASE METAL SULFIDE MINERALS IN ACID, NEUTRAL OR MILDLY ALKALINE CIRCUITS

[75] Inventor: D. R. Nagaraj, Stamford, Conn.

[73] Assignee: American Cyanamid Company, Stamford, Conn.

[21] Appl. No.: 641,658

[22] Filed: Aug. 17, 1984

[51] Int. Cl.<sup>4</sup> ..... B03D 1/02

[52] U.S. Cl. ..... 209/166; 252/61

[58] Field of Search ..... 209/166, 167; 252/61

[56] References Cited

U.S. PATENT DOCUMENTS

3,590,996 7/1971 Harris ..... 209/166  
3,590,998 7/1971 Collins et al. ..... 209/166

FOREIGN PATENT DOCUMENTS

643197 1/1979 U.S.S.R. ..... 209/166

Primary Examiner—Bernard Nozick  
Attorney, Agent, or Firm—Frank M. Van Riet; John M. Cornell

[57] ABSTRACT

A process for the beneficiation of base metal sulfide mineral values from base metal sulfide ores with selec-

tive rejection of gangue sulfide minerals at pH values of below about 10.0 by froth flotation is disclosed. The process includes the use of a new and improved collector which at pH values below 10.0 exhibits unexpectedly high collector activity for base metal sulfide minerals such as copper, lead and zinc and selectively rejects gangue sulfide minerals, such as pyrite and pyrrhotite. The collector for base metal sulfide mineral values for use in the process comprises at least one hydrocarboxy-carbonyl thionocarbamate compound having the formula:



wherein R<sup>1</sup> is C<sub>1</sub>-C<sub>6</sub> alkyl or phenyl and R<sup>2</sup> is C<sub>1</sub>-C<sub>8</sub> alkyl. In a preferred embodiment of the present invention, the froth flotation is conducted under acid pH conditions by adjusting the pH of the flotation slurry with sulfuric acid. The process provides excellent metallurgical recoveries of copper sulfide mineral values of high grade at a substantial reduction in lime consumption and reagents costs associated with prior art flotation separation methods. Bulk sulfide flotation methods are also disclosed.

13 Claims, No Drawings

PROCESS FOR THE FLOTATION OF BASE  
METAL SULFIDE MINERALS IN ACID, NEUTRAL  
OR MILDLY ALKALINE CIRCUITS

CROSS-REFERENCE TO RELATED  
APPLICATION

This application is related to commonly assigned, concurrently filed, U.S. application, Ser. No. 641,657, filed Aug. 17, 1984, of Y. L. Fu and S. S. Wang, entitled NEUTRAL HYDROCARBOXYCARBONYL THIONOCARBAMATE SULFIDE COLLECTORS.

BACKGROUND OF THE INVENTION

The present invention relates to froth flotation processes for recovery of metal values from base metal sulfide ores. More particularly, it relates to new and improved sulfide collectors comprising certain hydrocarboxycarbonyl thionocarbamate compounds which exhibit excellent metallurgical performance over a broad range of pH values.

Froth flotation is one of the most widely used processes for beneficiating ores containing valuable minerals. It is especially used for separating finely ground valuable minerals from their associated gangue or for separating valuable minerals from one another. The process is based on the affinity of suitably prepared mineral surfaces for air bubbles. In froth flotation, a froth or a foam is formed by introducing air into an agitated pulp of the finely ground ore in water containing a frothing or foaming agent. A chief advantage of separation by froth flotation is that it is a relatively efficient operation at a substantially lower cost than many other processes.

Current theory and practice state that the success of a sulfide flotation process depends to a great degree on the reagent(s) called collector(s) that impart(s) selective hydrophobicity to the value sulfide mineral that has to be separated from other minerals. Thus, the flotation separation of one mineral species from another depends upon the relative wettability of mineral surfaces by water. Typically, the surface free energy is purportedly lowered by the adsorption of heteropolar collectors. The hydrophobic coating thus provided acts in this explanation as a bridge so that the mineral particles may be attached to an air bubble. The practice of this invention is not, however, limited by this or other theories of flotation.

In addition to the collector, several other reagents are also necessary. Among these, the frothing agents are used to provide a stable flotation froth, persistent enough to facilitate the mineral separation, but not so persistent that it cannot be broken down to allow subsequent processing. The most commonly used frothing agents are pine oil, creosote and cresyllic acid and alcohols such as 4-methyl-2-pentanol, polypropylene glycols and ethers, etc.

Moreover, certain other important reagents, such as the modifiers, are also largely responsible for the success of flotation separation of sulfide minerals. Modifiers include all reagents whose principal function is neither collecting nor frothing, but one of modifying the surface of a mineral so that a collector either adsorbs to it or does not. Modifying agents can thus be considered as depressants, activators, pH regulators, dispersants, deactivators, etc. Often, a modifier may perform several functions simultaneously. Current theory and practice

of sulfide flotation again state that the effectiveness of all classes of flotation agents depends to a large extent on the degree of alkalinity or acidity of the ore pulp. As a result, modifiers that regulate the pH are of great importance. The most commonly used pH regulators are lime, soda ash and, to a lesser extent, caustic soda. In sulfide flotation, however, lime is by far the most extensively used. In copper sulfide flotation, which dominates the sulfide flotation industry, for example, lime is used to maintain pH values over 10.5 and more usually above 11.0 and often as high as 12 or 12.5. In prior art sulfide flotation processes, preadjustment of the pH of the pulp slurry to 11.0 and above is necessary, not only to depress the notorious gangue sulfide minerals of iron, such as pyrite and pyrrhotite, but also to improve the performance of a majority of the conventional sulfide collectors, such as xanthates, dithiophosphates, trithiocarbonates and thionocarbamates. The costs associated with adding lime are becoming quite high and plant operators are interested in flotation processes which require little or no lime addition, i.e., flotation processes which are effectively conducted at slightly alkaline, neutral or even at acid pH values. Neutral and acid circuit flotation processes are particularly desired because pulp slurries may be easily acidified by the addition of sulfuric acid, and sulfuric acid is obtained in many plants as a by-product of the smelters. Therefore, flotation processes which do not require preadjustment of pH or which provide for pH preadjustment to neutral or acid pH values using less expensive sulfuric acid are preferable to current flotation processes because current processes require pH preadjustment to highly alkaline values of at least about 11.0 using lime which is more costly.

To better illustrate the current problems, in 1980, the amount of lime used by the U.S. copper and molybdenum mining industry was close to 550 million pounds. For this industry lime accounted for almost 92.5% by weight of the total quantity of reagents used, and the dollar value of the lime used was about 51.4% of the total reagent costs for the industry, which amounted to over 28 million dollars.

As has been mentioned above, lime consumption in individual plants may vary anywhere from about one lb. of lime/metric ton of ore processed up to as high as 20 lbs. of lime/metric ton of ore. In certain geographical locations, such as South America, lime is a scarce commodity and the costs of transporting and/or importing lime have risen considerably in recent years. Still another problem with prior art highly alkaline processes is that the addition of large quantities of lime to achieve sufficiently high pH causes scale formation on plant and flotation equipment, thereby necessitating frequent and costly plant shutdowns for cleaning.

It is apparent, therefore, that there is a strong desire to reduce or eliminate the need for adding lime to sulfide flotation processes to provide substantial savings in reagents costs. In addition, reducing or eliminating lime in sulfide ore processing may provide other advantages by facilitating the operation and practice of unit operations other than flotation, such as slurry handling.

In the past, xanthates and dithiophosphates have been employed as sulfide collectors in froth flotation of base metal sulfide ores. A major problem with these conventional sulfide collectors is that at pH's below 11.0, poor rejection of pyrite or pyrrhotite is obtained. In addition, with decreasing pH the collecting power of these sul-

fide collectors also decreases, rendering them unsuitable for flotation in mildly alkaline, neutral or acid environments. This decrease in collecting power with decreasing pH, e.g., below about 11.0, requires that the collector dosage be increased many fold, rendering it generally economically unattractive. There are many factors which may account for the lowering of collector activity with decreasing pH. A collector may interact differently with different sulfide minerals at a given pH. On the other hand, poor solution stability at low pH, such as that exhibited by xanthates and trithiocarbonates may very well explain the observed weak collector behavior.

Efforts to overcome the above deficiencies led to the development of neutral derivatives of xanthates such as alkyl xanthogen alkyl formates generally illustrated by the formula:



The alkyl xanthogen alkyl formates are disclosed as sulfide collectors in U.S. Pat. No. 2,412,500. Other structural modifications of the general structure were disclosed later. In U.S. Pat. No. 2,608,572 for example, the alkyl formate substituents contain unsaturated groups. In U.S. Pat. No. 2,608,573, the alkyl formate substituents described contain halogen, nitrile and nitro groups. Bis alkyl xanthogen formates are described as sulfide collectors in U.S. Pat. No. 2,602,814. These modified structures have not found as much commercial application as the unaltered structures. For example, an alkyl xanthogen alkyl formate is currently commercially available under the trade name MINE-REC®A from the Minerec Corporation. MINE-REC®A, an ethyl xanthogen ethyl formate, as well as its higher homologs, still leave a lot to be desired at pH below 11.0 in terms of collecting power and pyrite rejection, as is more particularly described hereinafter.

Another class of sulfide collectors which have obtained some degree of commercial success in froth flotation are oily sulfide collectors comprising dialkylthionocarbamate or diurethane compounds having the general formula:



Several disadvantages are associated with the preparation and use of these compounds. In U.S. Pat. No. 2,691,635, a process for making dialkylthionocarbonates is disclosed. The three steps of the reaction sequence described are cumbersome and the final by-product is methyl mercaptan, an air pollutant which is costly to treat. In U.S. Pat. No. 3,907,854 an improved process for making dialkylthionocarbamate is described. Although good yields and high purity are claimed as the novel features of the process, it is noteworthy that a side product of the reaction is sodium 60 hydrosulfide, also a pollutant which requires special treatment for disposal. In U.S. Pat. No. 3,590,998 a thionocarbamate sulfide collector structure in which the N-alkyl substituent is joined by alkoxy carbonyl groups is disclosed. The preparation process described therein requires the use of expensive amino acid esters for the displacement reaction of the thio esters of xanthates. The by-products of this process are either

methyl mercaptan or sodium thioglycolate. In addition, this type of structurally modified thionocarbamate has enjoyed very little commercial success. As will become apparent from the disclosure of this invention below, dialkylthionocarbamates are weak collectors as the pH drops below certain values.

Accordingly, it is an object of the present invention to provide a new and improved sulfide collector and flotation process for the beneficiation of sulfide minerals employing froth flotation methods which does not require any pre-adjustment of pH to highly alkaline values.

It is another object of the present invention to provide a new and improved sulfide collector and froth flotation process for the beneficiation of sulfide minerals which provides selective recovery of sulfide metal values with selective rejection of pyrite, pyrrhotite and other gangue sulfides.

It is a further object of the present invention to provide a new and improved sulfide collector and flotation process for the beneficiation of sulfide minerals using froth flotation methods which employs a novel class of sulfide collector reagents which may be prepared and used without the formation of harmful by-products or environmental pollutants.

It is another object of the present invention to provide a flotation process for the beneficiation of sulfide ores at pH values of 10.0 or below using certain novel collectors containing novel donor atom combinations designed specifically for low pH flotation.

It is still another object of the present invention to provide a new and improved process for selective flotation of value sulfides in acid circuits, wherein inexpensive sulfuric acid is used to control the pH.

#### SUMMARY OF THE INVENTION

In accordance with these and other objects, the present invention, in one embodiment, provides a new and improved collector composition for beneficiating an ore containing sulfide minerals with selective rejection of pyrite, pyrrhotite and other gangue sulfides, said collector composition comprising at least one hydrocarboxy carbonyl thionocarbamate compound selected from compounds having the formula:



wherein R<sup>1</sup> and R<sup>2</sup> are each independently selected from saturated and unsaturated hydrocarbyl radicals, alkyl polyether radicals and aromatic radicals and such radicals optionally, and independently substituted with polar groups selected from halogen, nitrile and nitro groups. Particularly preferred hydrocarboxy carbonyl thionocarbamate sulfide collectors in accordance with the present invention comprise compounds of the formula wherein R<sub>1</sub> is C<sub>1</sub>-C<sub>6</sub> alkyl or aryl and R<sub>2</sub> is C<sub>1</sub>-C<sub>8</sub> alkyl.

Generally, and without limitation, the new and improved hydrocarboxy carbonyl thionocarbamate collectors of this invention may be used in amounts of from about 0.005 to 0.5 pounds per ton of ore, and preferably from about 0.01 to 0.1 pounds per ton of ore, to effectively selectively recover metal and mineral values from base metal sulfide ores while selectively rejecting pyrite and other gangue sulfides. The new and improved sulfide collectors of this invention may gener-

ally be employed independently of the pH of the pulp slurries. Again, without limitation, these collectors may be employed at pH values of from about 3.5 to 11.0, and preferably from about 4.0 to 10.0.

In accordance with another embodiment, the present invention provides a new and improved process for beneficiating an ore containing sulfide minerals with selective rejection of pyrite and pyrrhotite, said process comprising: grinding said ore to provide particles of flotation size, slurring said particles in an aqueous medium, conditioning said slurry with effective amounts of a frothing agent and a metal collector, and frothing the desired sulfide minerals preferentially over gangue sulfide minerals by froth flotation procedures; said metal collector comprising at least one hydrocarboxy carbonyl thionocarbamate compound selected from compounds having the formula given above.

In particularly preferred embodiments, a new and improved method for enhancing the recovery of copper sulfide minerals from an ore containing a variety of sulfide minerals is provided wherein the flotation process is performed at a controlled pH of less than or equal to 10.0, and the collector is added to the flotation cell.

The present invention therefore provides a new class of sulfide collectors and a new and improved process for froth flotation of base metal sulfide ores. The hydrocarboxy carbonyl thionocarbamate collectors and the process of the present invention unexpectedly provide superior metallurgical recovery in froth flotation separations as compared with conventional sulfide collectors, even at reduced collector dosages, and are effective under conditions of acid, neutral or mildly alkaline pH. In accordance with the present invention, a sulfide ore froth flotation process is provided which simultaneously provides for superior beneficiation of sulfide mineral values with considerable savings in lime consumption.

Other objects and advantages of the present invention will become apparent from the following detailed description and illustrative working examples.

#### DETAILED DESCRIPTION OF THE INVENTION

In accordance with the present invention, sulfide metal and mineral values are recovered by froth flotation methods in the presence of a novel sulfide collector, said collector comprising at least one hydrocarboxy carbonyl thionocarbamate compound of the formula:



wherein R<sup>1</sup> and R<sup>2</sup> are, independently, selected from saturated and unsaturated hydrocarbyl radicals, alkyl polyether radicals and aromatic radicals, said R<sup>1</sup> and R<sup>2</sup> radicals, optionally and independently being substituted by polar groups selected from halogen, nitrile and nitro groups. By hydrocarbyl is meant a radical comprised of 60 hydrogen and carbon atoms which includes straight or branched, saturated or unsaturated, cyclic or acyclic hydrocarbon radicals. The R<sup>1</sup> and R<sup>2</sup> radicals may be unsubstituted or optionally substituted by polar groups such as halogen, nitrile or nitro groups. In addition, R<sup>1</sup> and R<sup>2</sup> may independently be selected from alkyl polyether radicals of the formula:



wherein R<sup>3</sup> is C<sub>1</sub> to C<sub>6</sub> alkyl; Y is an ethylene or propylene group and n is an integer of from 1 to 4 inclusive.

5 R<sup>1</sup> and R<sup>2</sup> may also independently be selected from aromatic radicals such as benzyl, phenyl, cresyl and xylenyl radicals, and aralkyl or alkaryl radicals, or any of these aromatic radicals optionally substituted by the above-mentioned polar groups.

10 In preferred embodiments, the hydrocarboxy carbonyl thionocarbamate collectors of the above formula employed are those compounds wherein R<sup>1</sup> is selected from C<sub>1</sub> to C<sub>6</sub> alkyl, or aryl, and especially preferably are ethyl, isopropyl, or phenyl radicals; and R<sup>2</sup> is selected from C<sub>1</sub>-C<sub>8</sub> alkyl radicals, for example, methyl, ethyl, n-propyl, isopropyl, n-butyl, sec-butyl, isobutyl, n-amyl, isoamyl, n-hexyl, isohexyl, heptyl, n-octyl and 2-ethylhexyl.

15 Illustrative compounds within the above formula for use as sulfide collectors in accordance with the present invention include:

N-ethoxycarbonyl-O-methyl thionocarbamate, N-ethoxycarbonyl-O-ethyl thionocarbamate,

N-ethoxycarbonyl-O-(n-propyl)thionocarbamate,

N-ethoxycarbonyl-O-isobutyl thionocarbamate,

N-ethoxycarbonyl-O-(n-pentyl)thionocarbamate,

N-ethoxycarbonyl-O-(2-methylpentyl)thionocarbamate,

N-ethoxycarbonyl-O-allyl thionocarbamate,

N-ethoxycarbonyl-O-(2-methoxylethyl)thionocarbamate,

N-ethoxycarbonyl-O-(2-ethoxyethyl)thionocarbamate,

N-ethoxycarbonyl-O-(2-butoxyethyl)thionocarbamate,

N-propoxycarbonyl-O-propyl thionocarbamate,

N-phenoxy carbonyl-O-ethyl thionocarbamate; and

N-phenoxy carbonyl-O-isopropyl thionocarbamate, to name but a few.

20 The hydrocarboxy carbonyl thionocarbamate compounds of the present invention may be conveniently prepared, without forming polluting by-products, first, by reacting a corresponding chloroformate compound with ammonium, sodium or potassium thiocyanate to form an isothiocyanate intermediate, in accordance with equation (1) as follows:



25 30 35 40 45 50 wherein R<sup>1</sup> is the same as defined above and X is NH<sub>4</sub><sup>+</sup>, Na<sup>+</sup>, or K<sup>+</sup>.

Thereafter, the hydrocarboxy carbonyl isothiocyanate intermediate is reacted with an active hydroxyl compound in accordance with equation (2) as follows:



55 60 65 70 75 80 85 90 95 By active hydroxyl compound is meant any compound bearing an hydroxyl group which will readily react with the isothiocyanate to form the corresponding thionocarbamate. Illustrative active hydroxyl compounds include aliphatic alcohols, cyclic and acyclic, saturated and unsaturated, unsubstituted or substituted by polar groups such as halogen, e.g., chloro, bromo or iodo, nitrile and nitro groups; aryl alkanols such as

benzyl alcohols; ethoxylated and/or propoxylated alcohols and phenols.

The corresponding chloroformates for reaction with the ammonium, sodium or potassium thiocyanate in accordance with equation (1) above, may themselves be prepared by reaction of the corresponding aliphatic or aromatic alcohols with phosgene, in accordance with equation (3) as follows:



wherein  $R^4$  comprises any of the active hydroxyl compounds defined above. By way of further illustration, chloroformates made from ethoxylated or propoxylated alcohols may be prepared in accordance with this method, e.g.,



wherein  $R^5$  is  $C_1-C_6$  alkyl and  $n$  is 1 to 4 inclusive; as well as, aromatic alcohols such as phenols, cresols and xylenols, e.g.,



wherein  $R^6=H$  or  $CH_3$  and  $R^7=H$ ,  $CH_3$ ,  $Cl$ ,  $Br$ ,  $I$ ,  $-NO_2$  or  $-C\equiv N$ .

Referring again to the preparation of the new and improved hydrocarboxycarbonyl thionocarbamate sulfide collectors of the present invention shown in Equations (1) and (2) above, it is apparent that sodium chloride is the only innocuous side product in the reaction of equation (1). Moreover, in equation (2), the condensation of the isothiocyanate with the active hydroxyl compound is fast and complete and does not release any polluting by-product.

In accordance with the present invention, the above-described hydrocarboxycarbonyl thionocarbamates are employed as sulfide collectors in a new and improved froth flotation process which provides a method for enhanced beneficiation of sulfide mineral values from base metal sulfide ores over a wide range of pH values and more particularly under acidic, neutral, slightly alkaline and highly alkaline conditions.

In accordance with the present invention, the new and improved, essentially pH-independent, process for the beneficiation of mineral values from base metal sulfide ores comprises, firstly, the step of size-reducing the ore to provide ore particles of flotation size. As is apparent to those skilled in this art, the particle size to which an ore must be size reduced in order to liberate mineral values from associated gangue or non-values,

i.e., liberation size, will vary from ore to ore and may depend on several factors, such as, for example, the geometry of the mineral deposits within the ore, e.g., striations, agglomeration, comatrices, etc. In any event, as is common in this art, a determination that particles have been size reduced to liberation size may be made by microscopic examination. Generally, and without limitation, suitable particle size will vary from between about 50 mesh to about 400 mesh sizes. Preferably, the ore will be size-reduced to provide flotation sized particles of between about +65 mesh and about -200 mesh. Especially preferably for use in the present method are base metal sulfide ores which have been size-reduced to provide from about 14% to about 30% by weight of particles of +100 mesh and from about 45% to about 75% by weight of particles of -200 mesh sizes.

Size-reduction of the ores may be performed in accordance with any method known to those skilled in this art. For example, the ore can be crushed to -10 mesh size followed by wet grinding in a steel ball mill to specified mesh size or autogenous or semiautogenous grinding or pebble milling may be used. The procedure employed in size-reducing the ore is not critical to the method of this invention, as long as particles of effective flotation size are provided.

Preadjustment of pH is conveniently performed by addition of the modifier to the grind during the size reduction step.

The pH of the pulp slurry may be pre-adjusted to any desired value by the addition of either acid or base, and typically sulfuric acid or lime are used for this purpose, respectively. A distinct advantage of the present process is that the new and improved hydrocarboxycarbonyl thionocarbamate sulfide collectors employed in the process of this invention do not require any pre-adjustment of pH and generally the flotation may be performed at the natural pH of the ore pulp, thereby simplifying the process, saving costs and reducing lime consumption and related plant shut-downs. Thus, for example, good beneficiation has been obtained in accordance with the process of the present invention at pH values ranging between 3.5 and 11.0, and especially good beneficiation has been observed with pH values within the range of from about 4.0 to about 10.0 pH.

The size-reduced ore, e.g., comprising particles of liberation size, is thereafter slurried in aqueous medium to provide a floatable pulp. The aqueous slurry or pulp of flotation sized ore particles, typically in a flotation apparatus, is adjusted to provide a pulp slurry which contains from about 10 to 60% by weight of pulp solids, preferably 25 to 50% by weight and especially preferably from about 30% to about 40% by weight of pulp solids.

In accordance with a preferred embodiment of the process of the present invention, the flotation of copper, zinc and lead sulfides is performed at a pH of less than or equal to 10.0 and preferably less than 10.0. It has been discovered that in conducting the flotation at this pH, the new and improved hydrocarboxycarbonyl thionocarbamate collectors of the present invention exhibit exceptionally good collector strength, together with excellent collector selectivity, even at reduced collector dosages. Accordingly, in this preferred process, sulfuric acid is used to bring the pH of the pulp slurry to less than or equal to 10.0, if necessary.

In any event and for whatever reason, the pH of the pulp slurry may be pre-adjusted if desired at this time by any method known to those skilled in the art.

After the pulp slurry has been prepared, the slurry is conditioned by adding effective amounts of a frothing agent and a collector comprising at least one hydrocarboxycarbonyl thionocarbamate compound as described above. By "effective amount" is meant any amount of the respective components which provides a desired level of beneficiation of the desired metal values.

More particularly, any known frothing agent may be employed in the process of the present invention. By way of illustration such floating agents as straight or branched chain low molecular weight hydrocarbon alcohols, such as C<sub>6</sub> to C<sub>8</sub> alkanols, 2-ethyl hexanol and 4-methyl-2-pentanol, also known as methyl isobutyl carbinol (MIBC) may be employed, as well as, pine oils, cresylic acid, polyglycol or monoethers of polyglycols and alcohol ethoxylates, to name but a few of the frothing agents which may be used as frothing agent(s) herein. Generally, and without limitation, the frothing agent(s) will be added in conventional amounts and amounts of from about 0.01 to about 0.2 pounds of frothing agent per ton of ore treated are suitable.

The new and improved hydrocarboxycarbonyl thionocarbamate sulfide collectors for use in the process of the present invention may generally be added in amounts of from about 0.005 to about 0.5 pounds of collector per ton of ore and preferably will be added in amounts of from about 0.01 lbs. to about 0.3 lbs/ton of ore processed. In floatations wherein it is desired to selectively collect copper sulfide minerals and selectively reject iron sulfide minerals such as pyrite and pyrrhotite, as well as other gangue sulfides, the collectors will generally be added in amounts of from about 0.01 lbs/ton to about 0.1 lbs/ton of ore. In bulk sulfide floatations, higher levels of collector will be used, as will be more particularly described below.

Thereafter, in accordance with the process of the present invention, the conditioned slurry, containing an effective amount of frothing agent and an effective amount of collector comprising at least one hydrocarboxycarbonyl thionocarbamate compound, is subjected to a frothing step in accordance with conventional froth flotation methods to float the desired sulfide mineral values in the froth concentrate and selectively reject or depress pyrite and other gangue sulfides.

It has also been surprisingly discovered that, contrary to the conventional belief that a neutral, oily collector is most effective when it is added to the grind instead of to the flotation cell, the new and improved hydrocarboxycarbonyl thionocarbamate collectors of the present invention exhibit more efficient recovery when they are added to the flotation cell, as opposed to the grind. The novel collectors of this invention, although water-insoluble for all practical purposes, have the distinct advantage of being easily dispersible. The novel collectors when added to the flotation cell provide higher copper recovery in the first flotation stage together with improved copper recovery overall, indicating improved kinetics of flotation, to be more fully described hereinafter. Of course, the new and improved collectors may also be added to the grind in accordance with conventional methods, and improved value minerals recovery are still obtained.

Heretofore, the new and improved hydrocarboxycarbonyl thionocarbamate collectors and processes incorporating them of the present invention have been de-

scribed for use in those applications wherein it is desired to selectively concentrate or collect certain metal value sulfides, mainly those of copper, nickel lead and zinc from other gangue sulfides, e.g., pyrite and pyrrhotite, and other gangue materials, e.g., silicates, carbonates, etc. In certain cases, however, it may be desirable to collect all of the sulfides in an ore including sphalerite (ZnS) and the iron sulfides, i.e., pyrite and pyrrhotite, in addition to the copper sulfide minerals.

More particularly, there exist certain massive or complex sulfide ores which contain large amounts of iron sulfide minerals, such as pyrite and pyrrhotite. With these complex sulfide ores, flotation of the iron sulfide minerals is frequently desired to obtain the sulfur-values from these minerals, which after further processing can be made to yield sulfur and sulfur reagents. Under these circumstances, a bulk sulfide flotation is desired, i.e., a flotation wherein all of the sulfide minerals are floated and collected. Bulk sulfide floatations are also desired in order to benefit precious metals from precious metal-bearing pyrite and pyrrhotite minerals.

Often, however, these massive or complex sulfide ores not only contain several value metals as sulfides, such as copper, zinc, lead, nickel, cobalt, etc., but also contain, in close association therewith, gangue materials such as carbonates as well as silicas and siliceous materials.

These massive or complex sulfide ores are not uncommon and present a unique set of problems for froth flotation beneficiation. Bulk sulfide flotation for these ores cannot be successfully conducted under conventional flotation conditions, e.g., at pH values of >10.0, because pyrite and pyrrhotite values are depressed at high pH values. At pH values of 3.0 to 5.0, bulk sulfide flotation is high using conventional collectors, such as xanthates, but sulfuric acid is used as the modifier to reduce the pulp pH to these values. The carbonate gangue minerals present in these complex ores are acid-soluble and consequently large amounts of sulfuric acid are required, e.g. about 10-12 lbs/ton or ore, which is economically unattractive, and the use of sulfuric acid with ores containing alkaline earth metal carbonates such as calcite, dolomite, etc. results in the formation of large amounts of insoluble, alkaline earth metal sulfates, which causes very severe scaling on plant equipment, again necessitating frequent and costly plant shutdowns. At a pulp pH in the range of about 6.0 to 9.0, bulk sulfide flotation with conventional collectors such as xanthates is less than optimum.

It has been unexpectedly discovered that the new and improved hydrocarboxycarbonyl thionocarbamate collectors of this invention, under carefully specified conditions, provide optimum flotation of bulk sulfides from sulfide containing ores. In accordance with this aspect of the present invention, optimum bulk sulfide floatations are obtained by performing froth flotation under neutral or slightly alkaline pH values, and more particularly at a pH of 6.0 to 9.0, inclusive, and employing a larger amount of the hydrocarboxycarbonyl thionocarbamate collectors of this invention, namely at dosage levels of from about 0.1 to about 1.0 lbs/ton or, expressed differently, at levels of equal to or above about 0.3 moles/metric ton of ore.

After the bulk sulfide concentrate is prepared by flotation under these pH conditions and at the collector dosages specified, the value sulfides of copper, lead and zinc are separated from the large amount of iron sulfides present in the bulk concentrate, by a second stage flota-

tion at a higher pH, i.e. values above 9.0, whereby the value sulfides are collected and the iron sulfides are selectively depressed. In the past, xanthate collectors were employed in the bulk flotation at pH values of 3.0 to 5.0, and the second stage flotation wherein the iron sulfides are selectively depressed had to be run at a pH of about 11.0, because pyrite rejection for the xanthate collectors is poor below 11.0. As can be appreciated, considerable quantities of lime had to be added to modify the pH for this second stage flotation. Now, in accordance with this aspect of the present invention, using the hydrocarboxycarbonyl thionocarbamate collectors, bulk sulfide flotation is obtained at a higher pH of 6.0 to 9.0, and the lime consumption needed in the second stage of flotation, i.e., the separation of value metal sulfides from iron sulfides, is reduced. Moreover, the hydrocarboxycarbonyl thionocarbamate collectors of this invention are much stronger collectors for copper, lead and zinc in the pH range of 9.0 to 11.0, such that the second stage flotation may be carried out at pH values just sufficient to depress the iron sulfides, in which case there is no need to raise the pH beyond 11.0, thereby providing further savings in lime consumption.

Other objects and advantages provided by the new and improved collectors and process of this invention will become apparent from the following working Examples, which are provided by way of further illustration only to enable those skilled in this art to better understand and practice the present invention.

#### PREPARATION 1

##### Synthesis of Ethoxycarbonyl Isothiocyanate

A 2-liter three-necked round-bottomed flask fitted with a reflux condenser protected from the moisture by a drying tube containing anhydrous calcium sulfate, an addition funnel and a mechanical stirrer was mounted in a heating mantle. In the flask were placed 700 ml of dry acetonitrile and 194 grams of potassium thiocyanate. The mixture was heated, with stirring, to 70° C. and then the external heating was discontinued. To the mixture were added with stirring, 217 grams of ethyl chloroformate from the addition funnel in 40 minutes. An exothermic reaction set in. The mixture thickened and turned yellow. After the addition was completed, the temperature of the reaction mixture reached 77° C. The reaction mixture was stirred for 3 hours without any external heating. Thereafter, the reaction mixture was cooled to room temperature and the precipitate was removed by filtration. The precipitate cake was washed with dry acetonitrile. The filtrate and the washing were combined and concentrated by evaporation under reduced pressure. The residual liquid was distilled through a fractionating column. There were obtained 86.9 grams of ethoxycarbonyl isothiocyanate, a colorless liquid which boiled at 45° C./11 mm Hg or 48° C./12 mm Hg.

#### PREPARATION 2

##### Synthesis of N-Ethoxycarbonyl-O-Isopropyl Thionocarbamate

Forty ml of isopropyl alcohol were added to 10 grams of the ethoxycarbonyl isothiocyanate (PREPARATION 1) and the reaction solution was mixed well by stirring. After the exotherm was over, the reaction solution was let stand overnight and the progress of the reaction was monitored by the infrared spectrum of the reaction solution. Completion of the reaction was indicated by the disappearance of the absorption band at

1960-1990 cm<sup>-1</sup> for the N=C=S group. The excess of isopropyl alcohol was removed by stripping under reduced pressure to give an oil residue. Crystallization from petroleum ether (b.p. 35°-60° C.) yielded 13.1 grams of colorless crystals of N-ethoxycarbonyl O-isopropyl thionocarbamate, melting at 32°-33° C.

#### PREPARATION 3

##### Synthesis of N-Ethoxycarbonyl-O-Isobutyl Thionocarbamate

Forty ml of isobutyl alcohol were added to 10 grams of ethoxycarbonyl isothiocyanate of PREPARATION 1. After the reaction was complete, the excess isobutyl alcohol was removed by stripping under reduced pressure. There was obtained 15 grams of N-ethoxycarbonyl-O-isobutyl thionocarbamate which was a colorless oil.

#### PREPARATION 4

##### Synthesis of N-Phenoxy carbonyl-O-Ethyl Thionocarbamate

##### Summary of Reaction Sequence



A 250 ml round-bottomed three-necked flask was equipped with a reflux condenser, a thermometer, an addition funnel and a mechanical stirrer. To the reaction flask were added 100 ml of ethyl acetate and 9.7 grams of potassium thiocyanate. The mixture was stirred and heated. To the mixture were added, dropwise from the addition funnel, 15.7 grams of phenyl chloroformate in 30 minutes. After the exotherm was over, the reaction mixture was let stir for 1½ hours. (GC indicated that phenyl chloroformate was reacted completely). Ten ml of absolute ethyl alcohol were added. The reaction mixture was stirred and the progress of the reaction was monitored by IR until phenoxy carbonyl isothiocyanate had been consumed complete. Fifty ml of water were added to dissolve the solids. The reaction mixture was transferred to a 250 ml separatory funnel. The organic layer was collected. It was dried over MgSO<sub>4</sub> and filtered. The filtrate was concentrated by stripping off the volatiles. A solid weighing 20.4 grams was obtained. The solid was recrystallized from hexanes. The pure product melts at 81°-83° C.

The above synthesized hydrocarboxycarbonyl thionocarbamates were employed as collectors for a variety of sulfide ores and tested for beneficiation properties at a variety pH values and compared with prior art sulfide collector compounds. The other homologous an/or analogous hydrocarboxycarbonyl thionocarbamates employed in the following examples may be pre-

pared according to substantially identical preparation methods, substituting the appropriate corresponding active hydroxyl compounds to provide the R<sup>2</sup> group shown.

In each of the following Examples, the following general preparation and testing procedures were used:

The sulfide ores were crushed to -10 mesh sizes. An amount of the crushed ores of between about 500 to 2,000 grams was wet ground in a steel ball mill with a steel ball charge of 5.3 to 10.7 kg and at 50 to 75% solids for about 6 to 14 minutes or until a pulp having this size distribution indicated was obtained, generally about 10-20% +65 mesh, 14-30% +100 mesh and 40-80% -200 mesh. Lime and sulfuric acid were used as the pH modifiers to adjust the pH as required. These modifiers were generally added to the grind. The frother used was added to the grind in some tests and added to the flotation cell in others. In certain tests, 50% the collector was added to the grind, otherwise, the collector was added to the first and second stages of conditioning in the flotation cell.

The size reduced pulp, with or without frother and collector additives, was transferred to a Denver D12 rectangular flotation cell. The volume of the pulp was adjusted to 1200-2650 ml by adding water to provide a pulp density of about 20-45% solids and a pulp level in the cell at about 2 cm below the lip.

Collector and/or frother were added to the pulp while agitating at about 1100-1400 rpm. The pulp was conditioned for a period of two minutes and pH and temperature measurements were taken at that time. At the end of the two minutes conditioning, air was fed at about 5-7 liters/minute from a compressed air cylinder. The froth flotation was continued for about 3 minutes during which a first stage concentrate was collected. Thereafter the air was turned off and more collector and frother were added and the pulp was conditioned for an additional two minutes. After the second two minute conditioning step the air was turned on and a second stage concentrate was collected. The flotation times were predetermined to give a barren froth upon completion of flotation.

The first and second stage concentrates and tailings were filtered, dried, sampled and assayed for copper, iron and sulfur. Tap water at the required temperature was used in all tests. The abbreviation t is used to indicate a standard ton, e.g., 2000 lbs. and T represents a metric ton, e.g., 1000 kg. or 2204 lbs.

#### EXAMPLE 1

##### Natural pH Flotation

A U.S. southwestern copper ore with a copper head assay of 0.3% and 1.7% pyrite (FeS<sub>2</sub>) head assay was used in this series of tests. In this and all of the following examples, the gangue iron minerals such as pyrite, pyrrhotite, etc., are for the sake of convenience, simply referred to as pyrite. The principal copper minerals were chalcocite and chalcopyrite.

460 grams of the ore were ground for 8.5 minutes at 60% solids to obtain a pulp slurry with a size distribution of 17.5% +65 mesh, 35.2% +100 mesh and 41% -200 mesh. The natural pH of the pulp, i.e. without external addition of either lime or sulfuric acid pH modifiers, was found to be 5.5. The pulp was conditioned at 30% solids with the collector indicated and a frothing agent comprising 50/50 w/w MIBC/pine oil added at 0.08 lbs/ton of ore and first and second stage floatations conducted in accordance with the procedures outlined

above. The collectors employed and the results of the concentrate and tailings assays are set forth in TABLE 1, as follows:

TABLE 1

| Natural pH 5.5; Frother - 1:1 MIBC/pine oil 0.08 lbs/t<br>Head Assay: Cu - 0.3% FeS <sub>2</sub> - 1.7% |                                               |        |              |               |                            |
|---------------------------------------------------------------------------------------------------------|-----------------------------------------------|--------|--------------|---------------|----------------------------|
| Ex-<br>am-<br>ple                                                                                       | Collector                                     | Dosage | % Cu<br>Rec. | % Cu<br>Grade | % FeS <sub>2</sub><br>Rec. |
| A.                                                                                                      | Sodium Ethyl Xanthate                         | 0.054  | 18.6         | 0.7           | 2.1                        |
| B.                                                                                                      | Sodium Ethyl Xanthate                         | 0.200  | 82.8         | 4.0           | 89.7                       |
| C.                                                                                                      | Sodium Diethyl Dithiophosphate                | 0.100  | 66.6         | 3.3           | 64.4                       |
| D.                                                                                                      | Sodium diisobutyl dithiophosphinate           | 0.054  | 69.3         | 2.3           | 11.2                       |
| E.                                                                                                      | Ethyl Xanthogen Ethyl formate                 |        |              |               |                            |
|                                                                                                         | Batch 1                                       | 0.054  | 84.1         | 2.3           | 74.2                       |
|                                                                                                         | Batch 4                                       | 0.054  | 79.2         | 1.9           | 51.2                       |
|                                                                                                         | Batch 5                                       | 0.054  | 86.4         | 3.9           | 91.1                       |
| F.                                                                                                      | O-isopropyl-N-ethyl thiono-carbamate          | 0.054  | 73.2         | 2.7           | 57.1                       |
| G.                                                                                                      | O-isobutyl-N-ethyl thiono-carbamate           | 0.054  | 78.0         | 3.2           | 51.1                       |
| I.                                                                                                      | N-ethoxycarbonyl-O-isopropyl thiono-carbamate | 0.054  | 90.8         | 9.6           | 67.3                       |

<sup>a</sup>MINEREC ® A, Minerec Corporation, Baltimore, Md. U.S.A.

30

It is apparent that the conventional collectors shown in Examples A-G were much weaker than Example 1 of the present invention at this pH. The hydrocarboxy-carbonyl thiono-carbamate of Example 1 provided not only the maximum copper recovery for the collectors tested, but also maximum copper grade at an acceptable pyrite rejection.

#### EXAMPLES 2-3

40 For the following Examples a U.S. Southwestern copper-molybdenum ore was used which had a head assay of 0.458% copper and 2.2% pyrite. The ore contained chalcopyrite, chalcocite and covellite as the major copper minerals. The ore was steel ball milled at 63% solids to provide a pulp with a size distribution of about 16.4% +65 mesh, 30% +100 mesh and 43.8% -200 mesh. The natural pH of the ground ore pulp was 5.0. The frother used was 1:1 MIBC/pine oil added at 50 gms/metric ton (T). To make the comparisons more rigorous and meaningful, the collectors were dosed on a equimolar basis, 0.03 moles/T are approximately 0.01 lbs/ton. In addition, a selectivity/performance index was calculated for each of the collectors tested.

45 More particularly, the selectivity/performance index was defined and calculated in accordance with the equation:

$$I_{Cu} = \frac{(100 - \% \text{ Pyrite recovered})}{(100 - \% \text{ Copper recovered})^2}$$

55 The selectivity index for copper is a convenient method for measuring not only the copper recovery of a collector but also its selectivity for rejecting pyrite. For example, with this particular ore, if a 90% recovery for copper and a 50% recovery of pyrite can be accepted as optimum, then the optimum selectivity index for copper would be

60

65

$$I_{cu} = \frac{(100 - 50)}{(100 - 90)^2} = 0.5,$$

The collectors tested and the results obtained are set forth in Table 2 as follows:

TABLE 2

| Ex-<br>am-<br>ple | Collector                | Natural pH 5.0 (no lime);<br>Frother - 1:1 MIBC/pine oil at 50 g/T;<br>Collectors at 0.03 Mole/Ton (approx. 0.01 lb./t.) |                  |                               |                      |
|-------------------|--------------------------|--------------------------------------------------------------------------------------------------------------------------|------------------|-------------------------------|----------------------|
|                   |                          | %<br>Cu<br>Rec.                                                                                                          | %<br>Cu<br>Grade | %<br>FeS <sub>2</sub><br>Rec. | %<br>I <sub>cu</sub> |
|                   |                          | 33.2                                                                                                                     | 4.3              | 9.6                           | 0.02                 |
| H                 | Sodium isobutyl xanthate |                                                                                                                          |                  |                               |                      |

conventional collectors of Examples H-P. Examples 2 and 3 showed high copper recovery coupled with satisfactory pyrite rejection. Only the collectors of Examples 2 and 3 provided I<sub>cu</sub>'s close to the optimum 0.5 number.

## EXAMPLES 4-7

In the following Examples, tests were conducted employing the same ore as in Examples 2-3 with various collectors to determine if the superiority of the collectors of this invention was exhibited even at higher dosage levels and was not restricted to just one dosage. The collectors tested, the dosages and the results obtained are set forth in Table 3 as follows:

TABLE 3

| Example | Collector                                             | Mole/T<br>Dosage | % Cu.<br>Rec. | % Cu<br>Grade | % FeS <sub>2</sub><br>Rec. | I <sub>cu</sub> |
|---------|-------------------------------------------------------|------------------|---------------|---------------|----------------------------|-----------------|
| Q       | Ethyl Xanthogen<br>Ethyl Formate                      |                  |               |               |                            |                 |
|         | (Batch 1)                                             | 0.04             | 86.0          | 8.8           | 55.6                       | 0.227           |
|         | (Batch 3), pure                                       | 0.04             | 88.6          | 6.0           | 65.7                       | 0.261           |
| 4       | N-Ethoxycarbonyl-O—<br>isopropyl Thiono-<br>carbamate | 0.04             | 91.2          | 7.1           | 78.5                       | .277            |
| 5       | N-Ethoxycarbonyl-O—<br>Butyl Thionocarba-<br>mate     | 0.04             | 89.5          | 6.6           | 63.9                       | 0.330           |
| R       | Sodium ethyl Xan-<br>thate                            | 0.14             | 41.3          | 5.0           | 38.3                       | 0.018           |
| S       | Sodium diisobutyl<br>dithiophosphinate                | 0.14             | 59.0          | 7.7           | 24.0                       | 0.045           |
| T       | Ethyl xanthogen<br>Ethyl formate<br>(Batch 1)         | 0.14             | 86.0          | 8.1           | 91.5                       | 0.043           |
| U       | Sodium butyl tri-<br>thiocarbonate                    | 0.14             | 83.8          | 6.6           | 43.5                       | 0.216           |
| V       | Diallyl trithiocar-<br>bonate                         | 0.14             | 79.4          | 9.2           | 50.1                       | 0.117           |
| W       | Amyl allyl xanthate<br>ester                          | 0.14             | 75.4          | 9.8           | 40.4                       | 0.099           |
| 6       | N-Ethoxycarbonyl-O—<br>isopropylthiono-<br>carbamate  | 0.03             | 90.8          | 9.6           | 67.3                       | 0.389           |
| 7       | N—ethoxycarbonyl-O—<br>isopropylthionocar-<br>bamate  | 0.014            | 89.4          | 8.4           | 48.6                       | 0.456           |

|   |                                                    |      |     |      |       |    |
|---|----------------------------------------------------|------|-----|------|-------|----|
| I | O—isobutyl N—ethyl thio-<br>nocabamate             | 76.8 | 8.2 | 46.6 | 0.100 |    |
| J | O—isopropyl N—methyl thi-<br>onocabamate           | 67.7 | 5.8 | 38.8 | 0.059 | 45 |
| K | Ethyl Xanthogen Ethyl<br>Formate, Batch 1          | 84.6 | 9.2 | 50.0 | 0.211 |    |
|   | Ethyl Xanthogen Ethyl<br>Formate, Batch 1*         | 88.2 | 7.1 | 55.5 | 0.319 |    |
|   | Ethyl Xanthogen Ethyl<br>Formate, Batch 2          | 86.2 | 6.3 | 52.7 | 0.248 | 50 |
|   | Ethyl Xanthogen Ethyl<br>Formate, Batch 3, pure    | 85.7 | 6.4 | 56.9 | 0.212 |    |
| L | Sodium n-butyl trithio-<br>carbonate               | 58.8 | 6.4 | 16.9 | 0.049 |    |
| M | Isobutyl xanthogen ethyl<br>formate                | 85.6 | 7.7 | 38.2 | 0.297 | 55 |
| N | Isopropyl xanthogen ethyl<br>formate               | 86.2 | 6.5 | 65.5 | 0.180 |    |
| O | Isopropyl xanthogen<br>butyl formate               | 88.7 | 6.1 | 64.6 | 0.277 |    |
| P | Ethyl xanthogen phenyl<br>formate                  | 83.3 | 8.4 | 45.4 | 0.196 |    |
| 2 | N—Ethoxy carbonyl-O—isop-<br>ropyl thionocarbamate | 90.8 | 9.6 | 67.3 | 0.389 |    |
| 3 | N—Ethoxy carbonyl-O—amyl<br>thionocarbamate        | 91.1 | 6.7 | 58.3 | 0.525 |    |

\*This singular run gave unusually high copper recovery. All other data represent reproducible results.

The results of Table 2 clearly show the superiority of the collectors of this invention. Examples 2-3, over the

As demonstrated by the data of Table 3, the new and improved collectors of Examples 4 and 5 each exhibited better copper recovery and I<sub>cu</sub> value at a 0.04 mole/T dosage than the conventional collectors of Example Q. Moreover, conventional collectors R-W were inferior to Examples 4, 5, 6 and 7 even at dosages of 0.14 mole/T. These data show that at pH 5.0 the novel collectors of this invention outperform the conventional collectors even at sharply reduced dosage levels, e.g., one-fifth as much in Example 6 and one-tenth as much in Example 7.

## EXAMPLES 8-14

Using the same ore, the performance of conventional collectors and the collectors of this invention were compared with respect to hydrocarbon chain length and structural effects on performance against known dialkyl xanthogen formates. The collectors tested and the results obtained are set forth in Table 4 as follows:

TABLE 4

| Ex-<br>am-<br>ple                                                                                                                                                                                                          | Collector                                                                                                                                                                                                                 | Natural pH 5.0 (no lime);<br>Frother - 1:1 MIBC/pine oil at 50 g/T;<br>Collectors at 0.03 Mole/T (approx. 0.01 lb/t) |                  |                               |                 |
|----------------------------------------------------------------------------------------------------------------------------------------------------------------------------------------------------------------------------|---------------------------------------------------------------------------------------------------------------------------------------------------------------------------------------------------------------------------|----------------------------------------------------------------------------------------------------------------------|------------------|-------------------------------|-----------------|
|                                                                                                                                                                                                                            |                                                                                                                                                                                                                           | %<br>Cu<br>Rec.                                                                                                      | %<br>Cu<br>Grade | %<br>FeS <sub>2</sub><br>Rec. | I <sub>cu</sub> |
|                                                                                                                                                                                                                            |                                                                                                                                                                                                                           | Alkyl Xanthogen Alkyl (Phenyl) Formate                                                                               |                  |                               |                 |
| $\begin{array}{c} \text{S} \quad \text{O} \\ \parallel \quad \parallel \\ \text{R}_1-\text{O}-\text{C}-\text{S}-\text{C}-\text{OR}_2 \\ \text{R}_1 = \text{C}_2\text{H}_5, \text{R}_2 = \text{C}_2\text{H}_5. \end{array}$ |                                                                                                                                                                                                                           |                                                                                                                      |                  |                               |                 |
| Y                                                                                                                                                                                                                          | R <sub>1</sub> = i-C <sub>3</sub> H <sub>7</sub> , R <sub>2</sub> = C <sub>2</sub> H <sub>5</sub>                                                                                                                         | 84.6                                                                                                                 | 9.2              | 50.0                          | 0.211           |
| Z                                                                                                                                                                                                                          | R <sub>1</sub> = i-C <sub>4</sub> H <sub>9</sub> , R <sub>2</sub> = C <sub>2</sub> H <sub>5</sub>                                                                                                                         | 86.2                                                                                                                 | 6.3              | 52.7                          | 0.248           |
| AA                                                                                                                                                                                                                         | R <sub>1</sub> = i-C <sub>3</sub> H <sub>7</sub> , R <sub>2</sub> = n-C <sub>4</sub> H <sub>9</sub>                                                                                                                       | 85.7                                                                                                                 | 6.4              | 56.9                          | 0.212           |
| BB                                                                                                                                                                                                                         | R <sub>1</sub> = i-C <sub>3</sub> H <sub>7</sub> , R <sub>2</sub> = C <sub>6</sub> H <sub>5</sub>                                                                                                                         | 86.2                                                                                                                 | 6.5              | 65.5                          | 0.180           |
| CC                                                                                                                                                                                                                         | R <sub>1</sub> = C <sub>2</sub> H <sub>5</sub> , R <sub>2</sub> = C <sub>6</sub> H <sub>5</sub>                                                                                                                           | 85.6                                                                                                                 | 7.7              | 38.2                          | 0.297           |
|                                                                                                                                                                                                                            | $\begin{array}{c} \text{O} \quad \text{S} \\ \parallel \quad \parallel \\ \text{R}_1\text{O}-\text{C}-\text{NH}-\text{C}-\text{OR}_2 \\ \text{R}_1 = \text{C}_2\text{H}_5, \text{R}_2 = \text{C}_2\text{H}_5 \end{array}$ |                                                                                                                      |                  |                               |                 |
| 8                                                                                                                                                                                                                          | R <sub>1</sub> = C <sub>2</sub> H <sub>5</sub> , R <sub>2</sub> = C <sub>2</sub> H <sub>5</sub>                                                                                                                           | 83.2                                                                                                                 | 10.1             | 38.2                          | 0.219           |
| 9                                                                                                                                                                                                                          | R <sub>1</sub> = C <sub>2</sub> H <sub>5</sub> , R <sub>2</sub> = i-C <sub>3</sub> H <sub>7</sub>                                                                                                                         | 90.8                                                                                                                 | 9.6              | 67.3                          | 0.389           |
| 10                                                                                                                                                                                                                         | R <sub>1</sub> = C <sub>2</sub> H <sub>5</sub> , R <sub>2</sub> = i-C <sub>4</sub> H <sub>9</sub>                                                                                                                         | 90.6                                                                                                                 | 7.7              | 81.3                          | 0.212           |
| 11                                                                                                                                                                                                                         | R <sub>1</sub> = C <sub>2</sub> H <sub>5</sub> , R <sub>2</sub> = n-C <sub>4</sub> H <sub>9</sub>                                                                                                                         | 88.2                                                                                                                 | 10.2             | 49.6                          | 0.359           |
| 12                                                                                                                                                                                                                         | R <sub>1</sub> = C <sub>2</sub> H <sub>5</sub> , R <sub>2</sub> = C <sub>5</sub> H <sub>11</sub>                                                                                                                          | 91.1                                                                                                                 | 6.7              | 58.3                          | 0.525           |
| 13                                                                                                                                                                                                                         | R <sub>1</sub> = C <sub>6</sub> H <sub>5</sub> , R <sub>2</sub> = C <sub>2</sub> H <sub>5</sub>                                                                                                                           | 90.1                                                                                                                 | 6.8              | 71.9                          | 0.284           |
| 14                                                                                                                                                                                                                         | R <sub>1</sub> = C <sub>6</sub> H <sub>5</sub> , R <sub>2</sub> = i-C <sub>3</sub> H <sub>7</sub>                                                                                                                         | 90.9                                                                                                                 | 6.5              | 68.1                          | 0.384           |

The results shown in Table 4 demonstrate that, except for the diethyl homolog, all of the collectors of the present invention, e.g. Examples 8-14, showed better copper recovery than the corresponding conventional collectors substituted by the same R<sub>1</sub> and R<sub>2</sub> groups. The I<sub>cu</sub> values were also correspondingly better. The amyl homolog of Example 12 exhibited the best copper recovery and the best I<sub>cu</sub> value.

#### EXAMPLES 15-17

In the following Examples a South American copper-molybdenum ore was used. This ore contained 1.65% copper, 2.5% pyrite and 0.025% molybdenum. The copper was present as chalcocite, chalcopyrite, covellite, bornite, as well as some oxide copper minerals such

as malachite and cuprite. Although the ore contained a large amount of chalcopyrite, an appreciable amount of it was rimmed with chalcocite and covellite.

About 500 grams of the -10 mesh ore was wet ground for 13 minutes in a steel ball mill with a steel ball charge of 5.3 kg and at 63% solids to yield a pulp with a size distribution of 14% +100 mesh and 62% -200 mesh. 10.5 g/T of diesel oil were also added in all tests.

The natural pH of the ore pulp was 5.5. The standard 10 collector used for this ore is a mixture of a neutral alkyl xanthogen alkyl formate, e.g. ethyl xanthogen ethyl formate (MINERAC A), gasoline and 4-methyl-2-pentanol (MIBC) at a 60:30:10 ratio, respectively. The frother used is a polypropylene glycol monoalkylether, 15 such as polypropylene glycol monomethyl ether, added at 60 g/T. The standard collector in blended and unblended form was compared with the collectors of this invention at various dosage levels and the collectors were added to the flotation cell in the first and second 20 stages, in accordance with the flotation testing procedure outlined above. The test results are set forth in Table 5, as follows:

TABLE 5

| #  | Collector                                                     | Natural pH 5.5 (no lime, no H <sub>2</sub> SO <sub>4</sub> );<br>Frother - 60 g/T; |              |               |                            |
|----|---------------------------------------------------------------|------------------------------------------------------------------------------------|--------------|---------------|----------------------------|
|    |                                                               | Dosage<br>g/T                                                                      | % Cu<br>Rec. | % Cu<br>Grade | % FeS <sub>2</sub><br>Rec. |
| DD | 60/30/10 blend of ethyl xanthogen ethyl formate/gasoline/MIBC | 20                                                                                 | 66.1         | 6.7           | 69.5                       |
| EE | 60/30/10 blend of ethyl xanthogen ethyl formate/gasoline/MIBC | 40                                                                                 | 70.9         | 6.6           | 72.0                       |
| FF | 60/30/10 blend of ethyl xanthogen ethyl formate/gasoline/MIBC | 58                                                                                 | 72.9         | 6.2           | 76.8                       |
| 15 | N-Ethoxycarbonyl-O-isopropyl thionocarbamate                  | 20                                                                                 | 73.8         | 9.4           | 77.2                       |
| 16 | N-Ethoxycarbonyl-O-isopropyl thionocarbamate                  | 40                                                                                 | 76.4         | 8.3           | 80.8                       |
| 17 | N-Ethoxycarbonyl-O-isopropyl thionocarbamate                  | 58                                                                                 | 79.5         | 7.5           | —                          |
| GG | Ethyl xanthogen ethyl formate (Batch 1)                       | 20                                                                                 | 67.4         | 6.9           | 75.5                       |
| HH | Ethyl xanthogen ethyl formate (Batch 1)                       | 40                                                                                 | 72.3         | 6.7           | 75.8                       |
| II | Ethyl xanthogen ethyl formate (Batch 1)                       | 58                                                                                 | 68.4         | 7.2           | 70.5                       |

As demonstrated by the data of Table 5, the hydrocarboxycarbonyl thionocarbamate collectors of this invention shown in unblended form in Examples 15-17, were superior both in terms of percent copper recovered and grade as compared to the conventional neutral xanthogen formate collectors used either in pure or in blended form.

#### EXAMPLES 18-25

In the following Examples, the collectors of this invention in blended and unblended form were compared with the neutral xanthogen formate collectors on the same South American copper-molybdenum ore using the same testing procedures, however, this time the pH of the pulp slurry was adjusted to 4.0 by the addition of 5.0 Kg/T of sulfuric acid prior to conditioning and flotation testing. Again, the collectors were added to the flotation cell only, during the first and second conditioning steps. The collectors used and the results obtained are set forth in Table 6, as follows:

TABLE 6

| Cu = 1.65%, FeS <sub>2</sub> = 2.5%,<br>Sulfuric Acid 5.0 kg/T to pH 4.0<br>Frother Dow 1012 = 60 g/T |                                                                                     |               |              |               |                            |                 |
|-------------------------------------------------------------------------------------------------------|-------------------------------------------------------------------------------------|---------------|--------------|---------------|----------------------------|-----------------|
| #                                                                                                     | Collector                                                                           | Dosage<br>g/T | % Cu<br>Rec. | % Cu<br>Grade | % FeS <sub>2</sub><br>Rec. | I <sub>Cu</sub> |
| JJ                                                                                                    | Standard blend 60/30/10<br>Ethyl xanthogen ethyl<br>formate/gasoline/MIBC           | 5             | 33.4         | 3.4           | 15.8                       | 0.019           |
| KK                                                                                                    | Standard blend 60/30/10<br>Ethyl xanthogen ethyl<br>formate/gasoline/MIBC           | 10            | 46.7         | 4.5           | 21.1                       | 0.028           |
| LL                                                                                                    | Standard blend 60/30/10<br>Ethyl xanthogen ethyl<br>formate/gasoline/MIBC           | 20            | 80.4         | 6.7           | 79.4                       | 0.054           |
| MM                                                                                                    | Standard blend 60/30/10<br>Ethyl xanthogen ethyl<br>formate/gasoline/MIBC           | 30            | 89.6         | 7.2           | 91.5                       | 0.078           |
| NN                                                                                                    | Standard blend 60/30/10<br>Ethyl xanthogen ethyl<br>formate/gasoline/MIBC           | 40            | 90.1         | 7.2           | 92.2                       | 0.080           |
| OO                                                                                                    | Pure ethyl xanthogen<br>ethyl formate (Batch 3)                                     | 5             | 61.7         | 6.6           | 44.5                       | 0.038           |
| PP                                                                                                    | Pure ethyl xanthogen<br>ethyl formate (Batch 3)                                     | 15            | 88.5         | 8.8           | 88.2                       | 0.090           |
| QQ                                                                                                    | Pure ethyl xanthogen<br>ethyl formate (Batch 3)                                     | 20            | 90.6         | 8.4           | 93.4                       | 0.075           |
| 18                                                                                                    | Ethoxy carbonyl isopropyl thionocarbamate                                           | 5             | 68.7         | 6.6           | 52.3                       | 0.049           |
| 19                                                                                                    | Ethoxy carbonyl isopropyl thionocarbamate                                           | 10            | 89.7         | 7.9           | 92.1                       | 0.074           |
| 20                                                                                                    | Ethoxy carbonyl isopropyl thionocarbamate                                           | 20            | 93.2         | 7.4           | 91.7                       | 0.180           |
| 21                                                                                                    | 60/30/10 blend of<br>N—ethoxycarbonyl—O—<br>isopropyl thionocarbamate/gasoline/MIBC | 20            | 92.4         | 7.9           | 90.5                       | 0.163           |
| 22                                                                                                    | 36/54/10 blend of<br>N—ethoxycarbonyl—O—<br>isopropyl thionocarbamate/gasoline/MIBC | 20            | 91.6         | 9.1           | 90.3                       | 0.136           |
| 23                                                                                                    | N—Ethoxycarbonyl—O—iso-<br>butyl thionocarbamate                                    | 5             | 67.5         | 7.2           | 45.0                       | 0.052           |
| 24                                                                                                    | N—Ethoxycarbonyl—O—iso-<br>butyl thionocarbamate                                    | 10            | 89.8         | 9.0           | 87.7                       | 0.119           |
| 25                                                                                                    | N—Ethoxycarbonyl—O—iso-<br>butyl thionocarbamate                                    | 20            | 93.5         | 8.2           | 97.0                       | 0.072           |

Table 6 demonstrates that the collectors of this invention in pure form as shown in Examples 18–20 and 23–25 or in blended form as shown in Examples 21 and 22 exhibit stronger collector activity as compared to the standard xanthogen formate collector in blended or pure form at all of the dosages tested. Not only was the copper recovery of Examples 18–25 an average of about 3% higher with no loss in copper grade, but the recovery increase was obtained at a dosage much lower than that for the corresponding standard collectors. The dosage advantage for the hydrocarboxycarbonyl thionocarbamate collectors of this invention renders their use economically advantageous, e.g., better recovery with better grade at a cheaper reagents cost.

It should be mentioned that with this particular ore, the pyrite recoveries obtained were noticeably high and appeared to closely follow the copper recovery. A microscopic analysis disclosed that the pyrite in this particular ore at the grind employed was closely associated and/or rimmed with copper materials, such that a high copper recovery with this ore inevitably produced

high pyrite recovery. Even though high pyrite recoveries were observed for all of the collectors tested in Table 6, only the collectors of Examples 18–25 gave the highest I<sub>Cu</sub> values for this ore at pH 4.0. Moreover, as shown in Example 22 of Table 6, a blend containing only 36% of the hydrocarboxycarbonyl thionocarbamate collector gave a higher copper recovery than was obtained with the standard collectors.

#### EXAMPLES 26–27

The following examples were conducted using the same South American ore that was used in Examples 15–25 to investigate the sensitivity of the collectors of this invention to pH and to test their efficacy under strongly acidic conditions. The flotation conditions and reagents used in Examples 18–25 were used in the following tests. Collector dosage was 5 g/T. Sulfuric acid was used to adjust pulp pH to the pH value indicated. The collectors were each tested at pH 2.75 and 3.70, and the results obtained are set forth in Table 7 as follows:

TABLE 7

| Example | Collector                                       | pH   | H <sub>2</sub> SO <sub>4</sub><br>kg/T | Cu<br>Rec. | Cu<br>Grade | FeS <sub>2</sub><br>Rec. |
|---------|-------------------------------------------------|------|----------------------------------------|------------|-------------|--------------------------|
| 26      | N—Ethoxycarbonyl—O—<br>isobutyl thionocarbamate | 2.75 | 8.0                                    | 79.9       | 7.5         | 59.3                     |

TABLE 7-continued

| Example | Collector                                   | pH   | H <sub>2</sub> SO <sub>4</sub><br>kg/T | Cu<br>Rec. | Cu<br>Grade | FeS <sub>2</sub><br>Rec. |
|---------|---------------------------------------------|------|----------------------------------------|------------|-------------|--------------------------|
| 27      | N—Ethoxycarbonyl-O—isobutyl thionocarbamate | 3.70 | 5.2                                    | 80.1       | 8.4         | 81.0                     |
| RR      | Ethyl xanthogen ethyl formate (pure)        | 2.75 | 8.0                                    | 24.5       | 2.6         | 11.8                     |
| SS      | Ethyl xanthogen ethyl formate (pure)        | 3.70 | 5.2                                    | 19.1       | 2.5         | 8.5                      |

The data of Table 7 clearly demonstrate that the collectors of the present invention outperform by a large margin the conventional neutral xanthogen formate collectors even under strongly acidic conditions, and that the hydrocarboxycarbonyl thionocarbamate collectors of this invention are generally not sensitive to pH. As shown in Table 7, under identical conditions, the standard collectors provided only 20-25% copper recovery, whereas the novel collector of this invention

used was a 1:1 pine oil/MIBC mixture added at 50 g/T. Sulfuric acid was used to adjust the pH to the acid values indicated, and for a pH of 4.0, the sulfuric acid was added at about 1.7 kg/T.

15 The novel collectors were evaluated for collector strength and selectivity against a number of standard collectors under acid pH conditions using this particular ore. The collectors tested and the results obtained are set forth in Table 8 as follows:

TABLE 8

| pH 4.0, sulfuric acid 1.7 kg/T, Frother-1:1 pine oil/MIBC 50 g/T<br>Collector Dosage 0.01 Mole/T (approx. 2 g/T)<br>unless otherwise mentioned |                                                      |               |     |              |               |                            |                 |
|------------------------------------------------------------------------------------------------------------------------------------------------|------------------------------------------------------|---------------|-----|--------------|---------------|----------------------------|-----------------|
| Example                                                                                                                                        | Collector                                            | Dosage<br>M/T | pH  | % Cu<br>Rec. | % Cu<br>Grade | % FeS <sub>2</sub><br>Rec. | I <sub>Cu</sub> |
| TT                                                                                                                                             | Sodium diisobutyl dithiophosphate                    | 0.01          | 4.0 | 26.2         | 2.6           | 11.9                       | 0.016           |
| UU                                                                                                                                             | Sodium diisobutyl dithiophosphate                    | 0.03          | 4.0 | 53.1         | 4.5           | 34.5                       | 0.030           |
| VV                                                                                                                                             | Sodium diisobutyl dithiophosphate                    | 0.10          | 4.0 | 95.0         | 5.7           | 95.5                       | 0.180           |
| WW                                                                                                                                             | Sodium isobutyl xanthate                             | 0.01          | 4.0 | 20.0         | 1.9           | 10.6                       | 0.014           |
| XX                                                                                                                                             | Sodium isobutyl xanthate                             | 0.03          | 4.0 | 51.4         | 3.5           | 33.1                       | 0.028           |
| YY                                                                                                                                             | Sodium isobutyl xanthate                             | 0.10          | 4.0 | 94.9         | 5.1           | 99.5                       | 0.020           |
| ZZ                                                                                                                                             | Ethyl xanthogen ethyl formate (Batch 1)              | 0.01          | 4.0 | 92.3         | 6.7           | 93.1                       | 0.117           |
| AAA                                                                                                                                            | Ethyl xanthogen ethyl formate (Batch 1) pH 3.7       | 0.01          | 3.7 | 65.2         | 5.6           | 70.1                       | 0.025           |
| BBB                                                                                                                                            | Ethyl xanthogen ethyl formate (Batch 2)              | 0.01          | 4.0 | 91.0         | 6.0           | 96.4                       | 0.045           |
| CCC                                                                                                                                            | Ethyl xanthogen ethyl formate (Batch 2) pH 3.9       | 0.01          | 3.9 | 54.1         | 4.4           | 59.0                       | 0.019           |
| DDD                                                                                                                                            | Ethyl xanthogen ethyl formate (Batch 3), pure        | 0.01          | 4.0 | 94.8         | 5.3           | 93.4                       | 0.249           |
| 28                                                                                                                                             | N—Ethoxycarbonyl-O—isopropyl thionocarbamate         | 0.01          | 4.0 | 96.3         | 6.4           | 91.5                       | 0.621           |
| 29                                                                                                                                             | N—Ethoxycarbonyl-O—isopropyl thionocarbamate pH 3.90 | 0.01          | 3.9 | 94.9         | 5.8           | 92.3                       | 0.299           |
| 30                                                                                                                                             | N—Ethoxycarbonyl-O—isobutyl thionocarbamate          | 0.01          | 4.0 | 97.5         | 5.9           | 97.4                       | 0.426           |

shown in Examples 26 and 27 provided about an 80% 60 copper recovery. This result is probably due to the much greater hydrolytic stability of the present collectors over the standard collectors.

## EXAMPLES 28-30

The same U.S. Southwestern ore having a 0.458% copper and 2.2% pyrite head assay that was used in Examples 2-14 was used in these floatations. The frother

65 The results in Table 8 clearly demonstrate the superiority of the novel collectors of this invention (Examples 28-30) over the conventional collectors (examples TT-DDD) in terms of copper recovery, copper grade and selectivity index. It can be noted from Table 8 that with water-soluble, ionic collectors, dithiophosphate and xanthate, dosages that are 10 times more than that re-

quired for novel collectors had to be used to achieve the high copper recovery (approx. 95%) which is still lower than the recovery obtained with the novel collectors (97%). Even with the neutral collector, ethyl xanthogen ethyl formate, which is considered to be suitable for acid circuit applications, the copper recovery obtained is only in the range 91-95% (examples ZZ-DDD). Furthermore, the performance of this collector appears to be very sensitive to small fluctuations in pH; a slight decrease in pH from 4.0 to 3.9 or 3.7 drastically decreased copper recovery from 92.3 to 65.2% (compare Examples ZZ and AAA) and 91% to 54% (Examples BBB and CCC). Such is not the case with the novel collectors (compare Examples 28 and 29). This unusual stability with respect to pH provides a distinct advantage for the novel collectors over the conventional collectors, especially under actual plant conditions where pH fluctuations are inevitable.

## EXAMPLES 31-32

It is generally believed that a neutral, oily collector is most effective when it is added to the grind instead of to the flotation cell. This statement generally holds true if the collector is highly water-insoluble and indispersible. The hydrocarboxycarbonyl thionocarbamate collectors of this invention, although water-insoluble for all practical purposes, were known to be easily dispersible. Testing was devised to evaluate whether the dispersability of these collectors provided additional advantages in their use. In this connection, two flotations were performed, one wherein 50% of the collector was added to the grind and the other 50% was added to the flotation cell during stage two flotation, and a second wherein 50% of collector was added to the cell at stage 1 flotation and the other 50% to the cell at stage 2 flotation. The same ore and collectors were used herein as in Examples 4-14. The flotations were run and the concentrates and tailings were assayed for copper. The results obtained are set forth in Table 9 as follows:

TABLE 9

| Example | Collector/Addition Method                                                                      | Dosage M/T | Stage 1   |           | Stage 2   |           | Over all % Cu Rec. | Over all % Cu Grade |
|---------|------------------------------------------------------------------------------------------------|------------|-----------|-----------|-----------|-----------|--------------------|---------------------|
|         |                                                                                                |            | % Cu Rec. | % Cu Rec. | % Cu Rec. | % Cu Rec. |                    |                     |
| 31      | N-Ethoxycarbonyl-O-isobutyl thionocarbamate added 50% to grind + 50% to Stage 2 flotation.     | 0.01       | 22.1      | 74.2      | 96.3      | 5.6       |                    |                     |
| 32      | N-Ethoxycarbonyl-O-isobutyl thionocarbamate added 50% to Stage 1 and 50% to Stage 2 flotation. | 0.01       | 84.6      | 12.9      | 97.5      | 5.9       |                    |                     |

The results of Table 9 indicate that unexpectedly improved results are obtained by adding the collectors of the present invention to the flotation cell rather than to the grind. A comparison of Examples 31 with 32 shows that when the collectors of this invention are added to the cell only, overall copper recovery is increased, e.g. 97.5% Cu recovery for Example 32 as opposed to 96.3% cu recovery for Example 31. One possible explanation for this difference may be that although the novel collectors of the present invention are selective for iron, some of the collecting power of the collector for copper may be lost in the grinding step

due to adsorption of the collector to iron values in the steel ball milling/grinding apparatus.

It is interesting to note that the use of the novel collectors of this invention coupled with adding them to the flotation cell, instead of to the grind, provides an unexpected and rather dramatic improvement in the kinetics of flotation. More particularly, improved kinetics are demonstrated by better copper recoveries in the stage 1 flotation. As is readily understood by those skilled in this art, in a typical flotation process, the ore is floated to provide a rougher concentrate and tailings. The tailings are generally discarded and the rougher concentrate is reground, reconditioned and then subjected to cleaner flotation. This provides a cleaner concentrate and cleaner tailings. The cleaner concentrate is generally dried and delivered up for smelting or other further refining steps. The cleaner tails are then subjected to a scavenging flotation after reconditioning. Thereafter, the scavenging concentrate may be combined with the cleaner concentrate. The scavenged tailings may be combined with the main feed to the rougher flotation. In the reconditioning steps between the rougher, cleaner and scavenger flotation, the pH of the slurry is generally increased to provide better selectivity and copper recovery.

As shown by the data in Table 9, the novel collectors of this invention, when added to the cell, provided much higher and faster collector activity than when 50% of the collector was added to the grind. When the collector was added to the cell only, Example 32, about 84% of the copper floated in the stage 1 flotation in contrast to Example 31, wherein only 22.1% of the copper floated at stage 1. Improved kinetics of flotation yields a stage 1 rougher concentrate containing more copper and further indicates that reagent consumption may be reduced by judicious control of reagent feed and suggests that the number of cells in a flotation bank can be reduced. Throughput in the plant can also be increased.

## EXAMPLES 33-34

The following flotation Examples were conducted at a ph of about 8.3 using the Southwestern U.S. copper-molybdenum ore having a 0.458% copper and 2.2% pyrite head assay. The frother used was a 50/50 pine oil/MIBC blend added at 50 gms/T. The collectors were added at 0.01 mole/T (approximately 2 gms/T). Lime was added in an amount of 1.76 kg/T to adjust the pulp pH to about 8.3. Conventional flotation practice with this ore has been to provide an operating pH of

11.2-11.3 which requires the addition of about 4.412 kg/T of lime. The collectors tested and the results obtained are set forth in Table 10 as follows:

TABLE 10

| Exam-<br>ple | Collector                                        | pH 8.3, Lime 1.76 kg/T<br>Frother 1:1 pine oil/MIBC 50 g/T<br>Collector Dosage 0.01 M/T (approx. 2 g/T) |             |                          |                 |
|--------------|--------------------------------------------------|---------------------------------------------------------------------------------------------------------|-------------|--------------------------|-----------------|
|              |                                                  | Cu<br>Rec.                                                                                              | Cu<br>Grade | FeS <sub>2</sub><br>Rec. | I <sub>cu</sub> |
| EEE          | Ethyl xanthogen ethyl<br>formate (Batch 3, pure) | 84.2                                                                                                    | 5.4         | 28.6                     | 0.287           |
| FFF          | Ethyl xanthogen ethyl<br>formate (Batch 2)       | 85.9                                                                                                    | 6.7         | 29.6                     | 0.352           |
| 33           | N-Ethoxycarbonyl-O-isopropyl thionocarbamate     | 90.6                                                                                                    | 9.3         | 38.9                     | 0.688           |
| 34           | N-Ethoxycarbonyl-O-isobutyl thionocarbamate      | 90.8                                                                                                    | 7.7         | 46.2                     | 0.633           |

The results in Table 10 demonstrate the superiority of the hydrocarboxycarbonyl thionocarbamates of this invention over the conventional collector, ethyl xanthogen ethyl formate. Examples 33 and 34 provided about 5% higher copper recovery than was obtained with the conventional collector of Examples EEE and FFF, and the copper grades and I<sub>cu</sub> values were significantly higher also. These results were obtained at a 60% reduction in the lime consumption needed to process this ore, e.g. 1.76 kg/T for the present invention versus 4.412 kg/T for the conventional collectors.

## EXAMPLES 35-36

Identical flotation tests were performed using the same ore, frother and collector dosage used in Examples 33-34 with the exception that a pH of 7.2 was used. To obtain this pH about 1.18 kg/T of lime were added which represents a 73% reduction in lime consumption over the standard 4.412 kg/T lime dosage required to provide pH of 11.2-11.3 utilized in prior art flotations for this ore. The collectors tested and the results obtained are set forth in Table 11, as follows:

TABLE 11

| Exam-<br>ple | Collector                                        | pH 7.2, Lime 1.18 kg/T,<br>Frother 1:1 Pine oil; MIBC 50 g/T,<br>Collector dosage 0.01 M/T (approx. 2 g/T) |             |                          |                 |
|--------------|--------------------------------------------------|------------------------------------------------------------------------------------------------------------|-------------|--------------------------|-----------------|
|              |                                                  | Cu<br>Rec.                                                                                                 | Cu<br>Grade | FeS <sub>2</sub><br>Rec. | I <sub>cu</sub> |
| GGG          | Sodium diisobutyl di-thiophosphate               | 61.9                                                                                                       | 6.1         | 20.6                     | 0.055           |
| HHH          | Sodium isobutyl xanthate                         | 45.6                                                                                                       | 4.9         | 14.2                     | 0.029           |
| III          | Ethyl xanthogen ethyl<br>formate (Batch 1)       | 83.3                                                                                                       | 9.8         | 24.6                     | 0.270           |
| JJJ          | Ethyl xanthogen ethyl<br>formate (Batch 2)       | 86.0                                                                                                       | 7.7         | 30.8                     | 0.351           |
| KKK          | Ethyl xanthogen ethyl<br>formate (Batch 3, pure) | 86.0                                                                                                       | 7.6         | 33.5                     | 0.339           |
| 35           | N-Ethoxycarbonyl-O-isopropyl thionocarbamate     | 90.9                                                                                                       | 7.4         | 47.6                     | 0.632           |
| 36           | N-Ethoxycarbonyl-O-isobutyl thionocarbamate      | 89.9                                                                                                       | 7.4         | 54.8                     | 0.444           |

As demonstrated by the data of Table 11, even at a pH of 7.2, the new and improved hydrocarboxycarbonyl thionocarbamate collectors of this invention provided the best metallurgical performance compared to the conventional collectors, Examples GGG-KKK, in

terms of better copper recovery which was 4-45% higher than obtained with the conventional collectors, better grade of concentrate and higher I<sub>cu</sub> values.

## EXAMPLE 37

Identical flotation tests were performed using the same ore, frother and collector dosage as were used in Examples 33-36, with the exception that a pH of 10.0 was used. Lime was added at about 2.75 kg/T which represents a 38% reduction in lime consumption over the conventional 4.412 kg/T employed in the prior art processes. The results of testing at pH 10.0 are shown in Table 12 as follows:

TABLE 12

| Exam-<br>ple | Collector                                        | pH 10.0, Lime 2.75 Kg/T,<br>Frother - 1:1 pine oil/MIBC - 50 g/T,<br>Collector Dosage 0.01 M/T (approx. 2 g/T) |             |                          |                 |
|--------------|--------------------------------------------------|----------------------------------------------------------------------------------------------------------------|-------------|--------------------------|-----------------|
|              |                                                  | Cu<br>Rec.                                                                                                     | Cu<br>Grade | FeS <sub>2</sub><br>Rec. | I <sub>cu</sub> |
| LLL          | Ethyl xanthogen ethyl<br>formate (pure, Batch 3) | 90.8                                                                                                           | 6.5         | 76.0                     | 0.284           |
| MMM          | Ethyl xanthogen ethyl<br>formate (Batch 2)       | 88.7                                                                                                           | 7.3         | 52.6                     | 0.373           |
| 37           | N-Ethoxycarbonyl-O-isobutyl thionocarbamate      | 89.7                                                                                                           | 8.2         | 31.8                     | 0.640           |

The results of Table 12 indicate, that at a pH of 10.0, the hydrocarboxycarbonyl collector of Example 37 provided about 1% lower copper recovery than the conventional collector of Example, but exhibited a dramatically better selectivity against pyrite, e.g. only 32% pyrite recovery for Example 37 as compared with 76% for Example LLL, which is reflected in the higher I<sub>cu</sub> values.

## EXAMPLES 38-43

In the following Examples, a Southwestern U.S. copper-molybdenum ore was used which had a head assay for copper of about 0.778% and for pyrite of about 5.7%. This ore was one of the most complicated of all of the ores tested in terms of complex mineralogy, low overall copper recovery, high lime consumption, and frothing problems. The ore contained predominantly chalcocite, however, the pyrite in the ore was excessively rimmed and disseminated with chalcocite and covellite. Pyrite separation in the rougher flotation was therefore not possible and was not attempted.

880 gms of the ore were conditioned with 500 gm/T of ammonium sulfide and ground for six minutes at 55.5% solids to obtain a pulp with the size distribution of 17.4% +65 mesh, 33% +100 mesh and 47.4% -200 mesh. The pulp was conditioned at 1500 rpm and 20.4% solids.

The standard operating pH for this ore is 11.4-11.5 using as a standard collector N-ethyl-O-isopropyl thionocarbamate. The lime consumption required to provide an operating pH of 11.4-11.5 is about 3.07 kg/T. The standard frother is cresylic acid added at about 150 gms/T.

The collectors were tested at the dosages and under the conditions indicated, and the results are set forth in Table 13, as follows:

TABLE 13

| Head Assay Cu = 0.778%, FeS <sub>2</sub> = 5.7%,<br>Frother - Cresylic Acid - 150 g/T, -<br>Collector Dosage and pH - see below |                                              |               |      |              |              |               |                            |                 |
|---------------------------------------------------------------------------------------------------------------------------------|----------------------------------------------|---------------|------|--------------|--------------|---------------|----------------------------|-----------------|
| Example                                                                                                                         | Collector                                    | Dosage<br>M/T | pH   | Lime<br>Kg/T | % Cu<br>Rec. | % Cu<br>Grade | % FeS <sub>2</sub><br>Rec. | I <sub>cu</sub> |
| NNN                                                                                                                             | N-ethyl O-isopropyl thiono-carbamate         | 0.105         | 8.0  | 0.23         | 74.3         | 10.3          | 62.2                       | 0.057           |
| OOO                                                                                                                             | N-ethyl O-isopropyl thiono-carbamate         | 0.210         | 8.0  | 0.23         | 68.6         | 8.3           | 73.5                       | 0.027           |
| PPP                                                                                                                             | N-ethyl O-isopropyl thiono-carbamate         | 0.105         | 9.0  | 0.74         | 78.2         | 9.7           | 62.0                       | 0.080           |
| QQQ                                                                                                                             | N-ethyl O-isopropyl thiono-carbamate         | 0.210         | 9.0  | 0.85         | 79.1         | 8.9           | 71.5                       | 0.065           |
| RRR                                                                                                                             | N-ethyl O-isopropyl thiono-carbamate         | 0.105         | 11.5 | 3.07         | 57.8         | 15.4          | 24.4                       | 0.042           |
| SSS                                                                                                                             | N-ethyl O-isopropyl thiono-carbamate         | 0.210         | 11.5 | 3.07         | 81.0         | 11.6          | 54.8                       | 0.126           |
| 38                                                                                                                              | N-Ethoxycarbonyl-O-isopropyl thionocarbamate | 0.105         | 8.0  | 0.23         | 80.4         | 9.4           | 75.0                       | 0.065           |
| 39                                                                                                                              | N-Ethoxycarbonyl-O-isopropyl thionocarbamate | 0.210         | 8.0  | 0.23         | 81.5         | 7.8           | 92.5                       | 0.022           |
| 40                                                                                                                              | N-Ethoxycarbonyl-O-isopropyl thionocarbamate | 0.105         | 9.0  | 0.74         | 80.1         | 9.6           | 69.1                       | 0.078           |
| 41                                                                                                                              | N-Ethoxycarbonyl-O-isobutyl thionocarbamate  | 0.105         | 8.0  | 0.23         | 78.8         | 8.3           | 85.6                       | 0.032           |
| 42                                                                                                                              | N-Ethoxycarbonyl-O-isobutyl thionocarbamate  | 0.210         | 8.0  | 0.23         | 82.4         | 7.8           | 94.5                       | 0.018           |
| 43                                                                                                                              | N-Ethoxycarbonyl-O-isobutyl thionocarbamate  | 0.105         | 9.0  | 0.70         | 82.6         | 8.8           | 79.6                       | 0.067           |

It is evident from the results in Table 13 that the novel collectors of this invention (Examples 38-40 and 42-43) returned superior metallurgy at pH 8.0 and 9.0 compared with the standard collector (Examples NNN-SSS) at pH 11.5. By using the novel collectors at pH 8.0 or 9.0, acceptable metallurgy can be achieved at dramatically reduced lime consumption (7.5% of the total lime consumption to give pH 8.0 and 25% of the total to give pH 9.0) and reduced collector dosage (0.105 M/T instead of 0.210 M/T required for standard collector at pH 11.5).

transferred to the flotation cell and conditioned at 1100 rpm and 32% solids.

This ore was used for further flotation tests in mildly alkaline circuits with the novel collectors of this invention. The standard collector scheme is composed of about 30-40 g/T of sodium isopropyl xanthate and 2.5 g/T of di(secbutyl) dithiophosphate and the standard flotation pH is 10.5. The lime consumption at this pH is about 0.53 Kg/T. The standard frother is 1:1:1 polypropylene glycol monomethylether/MIBC/pine oil at 20-25 g/T. The collectors tested and the results obtained are set forth in Table 14 as follows:

TABLE 14

| Head Cu = 1.85%, FeS <sub>2</sub> = 4.2%,<br>Frother - 1:1:1 Dow 250/MIBC/pine oil - 25.5 g/T,<br>Collector dosage and pH - see below |                                              |               |      |              |              |               |                            |                 |
|---------------------------------------------------------------------------------------------------------------------------------------|----------------------------------------------|---------------|------|--------------|--------------|---------------|----------------------------|-----------------|
| Example                                                                                                                               | Collector                                    | Dosage<br>M/T | pH   | Lime<br>Kg/T | % Cu<br>Rec. | % Cu<br>Grade | % FeS <sub>2</sub><br>Rec. | I <sub>cu</sub> |
| TTT                                                                                                                                   | Sodium isopropyl xanthate                    | 0.19          | 8.0  | 0.11         | 60.0         | 16.0          | 62.0                       |                 |
| UUU                                                                                                                                   | Sodium isopropyl xanthate                    | 0.19          | 9.0  | 0.29         | 79.3         | 16.0          | 83.1                       | 0.04            |
| VVV                                                                                                                                   | Sodium isopropyl xanthate                    | 0.19          | 10.5 | 0.53         | 85.5         | 15.6          | 88.1                       | 0.057           |
| XXX                                                                                                                                   | Sodium isopropyl xanthate                    | 0.125         | 10.5 | 0.53         | 84.4         | 11.8          | 86.2                       | 0.057           |
| 44                                                                                                                                    | N-Ethoxycarbonyl-O-isopropyl thionocarbamate | 0.125         | 9.0  | 0.25         | 84.2         | 14.5          | 78.0                       | 0.088           |
| 45                                                                                                                                    | N-Ethoxycarbonyl-O-isobutyl thionocarbamate  | 0.0625        | 8.0  | 0.12         | 86.3         | 17.3          | 55.1                       | 0.241           |
| 46                                                                                                                                    | N-Ethoxycarbonyl-O-isobutyl thionocarbamate  | 0.125         | 8.0  | 0.12         | 84.5         | 16.6          | 55.2                       | 0.187           |
| 47                                                                                                                                    | N-Ethoxycarbonyl-O-isobutyl thionocarbamate  | 0.125         | 9.0  | 0.24         | 89.9         | 14.4          | 88.9                       | 0.109           |

## EXAMPLES 44-47

A South American Cu-Mo ore which contained 1.844% Cu and 4.2% pyrite was used in the following tests. The copper minerals were predominantly chalcocite, chalcopyrite, covellite and bornite.

510 g of the ore was wet ground for 7.5 min. at 68% solids to obtain a pulp with the size distribution of 24.7% +65M, 38.3% +100M and 44% -200M. 2.5 g/T of di-sec butyl dithiophosphate was added to the grind in all of the test. Lime was also added to the grind to obtain the required pH in flotation. The pulp was

The results given in Table 14 demonstrate that the novel collectors of this invention show an excellent performance, both in terms of copper recovery (with no loss in Cu grade) and pyrite rejection at a reduced lime consumption and reduced collector dosage. Most importantly, the standard collector gave an unacceptably low copper recovery at pH 8.0 even with an increased collector dosage.

## EXAMPLE 48

In the earlier examples, it has been demonstrated that the new and improved hydrocarboxycarbonyl thionocarbamate collectors of the present invention exhibit superior performance at reduced or no lime consumption and at reduced dosages of collector as compared with a large number of conventional collectors on a variety of ores in the rougher or first stage flotation. In actual practice, the rougher concentrate is

parison. Additional collector was added in Example 48, in the stage 2 cleaner flotation, because it appeared that the amount added in the rougher flotation was not enough to carry over into the cleaner flotation. The standard collector carried over and was present in sufficient quantities in the second stage flotation, so that no additional collector was added in the second stage control.

The results obtained are set forth in Table 15, as follows:

TABLE 15

| EXAMPLE                    | CLEANER FLOTATIONS        |                                             |
|----------------------------|---------------------------|---------------------------------------------|
|                            | FFFF                      | 48                                          |
| Collector                  | Sodium isopropyl xanthate | N-Ethoxycarbonyl-O-Isobutyl thionocarbamate |
| <u>A. FIRST STAGE</u>      |                           |                                             |
| <u>Rougher Flotation</u>   |                           |                                             |
| Collector dosage, g/T      | 30.0                      | 12.8                                        |
| pH                         | 10.5                      | 8.2                                         |
| lime used, Kg/T            | 0.608                     | 0.108                                       |
| Recovery, %                |                           |                                             |
| Cu                         | 86.9                      | 88.1                                        |
| FeS <sub>2</sub>           | 90.9                      | 63.7                                        |
| Mo                         | 64.0                      | 55.6                                        |
| Grade, %                   |                           |                                             |
| Cu                         | 18.30                     | 21.30                                       |
| Fe                         | 20.70                     | 16.40                                       |
| <u>B. SECOND STAGE</u>     |                           |                                             |
| <u>Cleaner Flotation</u>   |                           |                                             |
| Collector dosage, g/T      | —                         | 4.2                                         |
| pH                         | 11-11.6                   | 8.7-9.6                                     |
| Lime used, Kg/T            | 0.343                     | 0.118                                       |
| Grade of Cleaner Conc., %  |                           |                                             |
| Cu                         | 39.4                      | 41.9                                        |
| Fe                         | 22.2                      | 18.6                                        |
| Mo                         | 0.56                      | 0.58                                        |
| TOTAL COLLECTOR ADDED, g/T | 30.0                      | 17.0                                        |
| TOTAL LIME ADDED, kg/T     | 0.951                     | 0.226                                       |
| TOTAL FROTHER ADDED, g/T   | 38.0                      | 39.0                                        |

cleaned in one or more stages to obtain a high grade copper minerals or copper-molybdenum minerals concentrate for further treatment for metal production.

The following examples illustrate the use of the new and improved hydrocarboxycarbonyl thionocarbamate collectors in cleaner flotation systems to provide higher copper grade concentrates for use in smelters or the like.

In the following examples, the same ore was used as that for Examples 44-47. The first stage or rougher flotation was performed in accordance with the methods of Examples 1-47. The concentrate was filtered and dried and then reground to form a pulp of approximately 40% solids. The pH of the reground was adjusted with lime and more collector and frother were added as needed. The reground pulp was conditioned and re-floated as before with the rougher concentrate to provide cleaner concentrate and cleaner tails. The cleaner tails were scavenged at gradually higher pH values, with or without further addition of collector and frother, and finally scavenged at a pH of greater than 11.0 with additional collector to float any remaining copper minerals, and each stage product was separately analyzed.

The following Table 15 shows the results obtained by subjecting the ore to a rougher stage flotation and a second stage or cleaner flotation, using a standard sodium isopropyl xanthate collector at pH 11.0 for com-

15  
45  
50  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985

ery in the rougher flotation, e.g., 63.7% as compared with the standard collector, e.g., 90%. Moreover, the copper recovery in the rougher flotation provided by the collector of this invention in Example 48 was higher than that obtained with the standard collector using less than half the dosage of the standard collector in the rougher flotation.

## EXAMPLE 49

## Bulk Sulfide Flotation

An Eastern/Southern U.S. copper-zinc-pyrite-pyrrhotite ore was used in the following flotation tests. It contained about 0.5-0.7% copper as chalcopyrite, 0.9% zinc and 30-35% iron as pyrrhotite and pyrite. The ore also contained a large amount of carbonate gangue minerals, such as calcite, dolomite, etc., in addition to the usual silicate or siliceous type gangue.

The ball mill discharge from an operating plant was used for all of the tests. The pulp contained ore particles of about 40%-200 mesh. About 4 liters of pulp were modified with 1-10 lbs/ton of concentrated sulfuric acid at 25% solids for 30 secs at 1800 rpm. The collector and frother were then added and the pulp was conditioned for 2 minutes. Flotation was carried out for 4 minutes with natural air flow rate at 1800 rpm agitation and a first stage concentrate was collected. The pulp was then conditioned for 30 seconds with additional frother and a second stage flotation concentrate was collected for 4 minutes. The first stage and second stage concentrates and the tails were filtered, dried and assayed for copper, iron, sulfur and zinc.

The results are given in Table 16, below. The conventional collector was sodium ethyl xanthate and the frother was a polypropylene glycol (OP 515 of Orepreg Inc.).

5 nyl-O-alkyl thionocarbamates, other hydrocarboxycarbonyl thionocarbamates of the above formula may be used as the sulfide collector herein, such as N-cyclohexoxycarbonyl-O-alkyl thionocarbamates N-(3-butene)1-oxycarbonyl-O-alkyl thionocarbamates, N-alkoxycarbonyl-O-arylthionocarbamates and N-aryloxycarbonyl-O-aryl thionocarbamates to name but a few. Moreover, as has been mentioned above, the process may be practiced using as the collector component mixtures of two or more of the hydrocarboxycarbonyl thionocarbamates, as well as mixtures of at least one hydrocarboxycarbonyl thionocarbamate collector in combination with another known collector which may be selected from, for example

10 (a) xanthates of xanthate esters, e.g.



15 respectively;

(b) dithiophosphates



20 (c) thionocarbamates, e.g.



25 (d) dithiophosphinates, e.g.

30 35 TABLE 16

| BULK SULFIDE FLOTATION                                  |                                             |                         |                                                  |             |      |      |          |      |      |
|---------------------------------------------------------|---------------------------------------------|-------------------------|--------------------------------------------------|-------------|------|------|----------|------|------|
| Head assay: Cu = 0.677, Zn = 1.00, Fe = 33.2, S = 19.24 |                                             |                         |                                                  |             |      |      |          |      |      |
| Frother = 35 g/T                                        |                                             |                         |                                                  |             |      |      |          |      |      |
| Example                                                 | Collector                                   | Collector Dosage<br>g/T | H <sub>2</sub> SO <sub>4</sub><br>Dosage<br>kg/T | Recovery, % |      |      | Grade, % |      |      |
|                                                         |                                             |                         |                                                  | Cu          | Fe   | Zn   | S        | Cu   | Fe   |
| GGGG                                                    | Sodium Ethyl Xanthate                       | 107.6                   | 4.88                                             | 96.5        | 90.6 | 56.1 | 97.5     | 1.22 | 53.0 |
| HHHH                                                    | Sodium Ethyl Xanthate                       | 101.2                   | 4.59                                             | 94.3        | 87.4 | 52.4 | 96.2     | 1.25 | 54.2 |
| IIII                                                    | Sodium Ethyl Xanthate                       | 70.0                    | 4.24                                             | 92.0        | 88.1 | 43.3 | 96.1     | 1.15 | 54.4 |
| 49                                                      | N-Ethoxycarbonyl-O-isobutyl thionocarbamate | 77.0                    | 1.87                                             | 95.0        | 92.2 | 55.1 | 98.3     | 1.08 | 54.6 |

The results in Table 16 demonstrate that the hydrocarboxycarbonyl thionocarbamate collectors of this invention in Example 49 provide essentially equivalent metallurgy in bulk sulfide flotation at about 25% lower dosage and about 62% lower sulfuric acid consumption, as compared with the conventional collector of Examples GGGG-IIII.

The foregoing examples demonstrate the significant improvements and advantages achieved with the new and improved hydrocarboxycarbonyl thionocarbamate collectors of this invention over a number of conventional collectors known to those skilled in this art.

Although the present process has been described with reference to certain preferred embodiments, modifications or changes may be made therein by those skilled in this art. For example, instead of N-ethoxycarbonyl-O-alkyl thionocarbamates and N-phenoxyacar-

55

(e) dithiocarbamates and derivatives thereof, e.g.



respectively;

(f) trithiocarbonates and derivatives thereof, e.g.,



respectively; and

60

65

(g) mercaptans, e.g.,

 $R^{10}SH$ ;

wherein in each of (a)-(e) above  $R^8$  is  $C_1-C_6$  alkyl and  $R^9$  is  $C_1-C_6$  alkyl, aryl or benzyl, and  $R^{11}$  is hydroxy or  $R^8$  and in (f)  $R^{10}$  is  $C_1-C_{12}$  alkyl.

In place of copper mineral values, the process of the present invention may be used to beneficiate other sulfide mineral and metal values from sulfide ores, including, for example, lead, zinc, nickel, cobalt, molybdenum, iron, as well as precious metals such as gold, silver, platinum, palladium, rhodium, iridium, ruthenium, and osmium. All such obvious modifications or changes may be made herein by those skilled in this art, without departing from the scope and spirit of the present invention as defined by the appended claims.

What is claimed is:

1. A process for the beneficiation of base metal sulfide minerals from base metal sulfide ores with selective rejection of gangue sulfide minerals at a pH value of less than 10.0, said process comprising:

- (a) providing an aqueous pulp slurry of finely divided, liberation-sized ore particles having a pH of less than 10.0;
- (b) conditioning said pulp slurry with effective amounts of a frothing agent and a metal collector, respectively, said metal collector comprising at least one hydrocarboxycarbonyl thionocarbamate compound having the formula:



wherein  $R^1$  is  $C_1-C_6$  alkyl and  $R^2$  is  $C_1-C_8$  alkyl;

(c) thereafter, frothing the base metal sulfide minerals by froth flotation;

(d) and recovering the base metal sulfide minerals.

2. A process as defined in claim 1, wherein said metal collector is added in an amount of from about 0.005 to about 0.1 lbs/tons of ore.

3. A process as defined in claim 1, wherein the pH of said aqueous pulp slurry is between about 3.5 and 10.0.

4. A process as defined in claim 1, wherein in said metal collector  $R^1$  is ethyl and  $R^2$  is isopropyl.

5. A process as defined in claim 1, wherein in said metal collector  $R^1$  is ethyl and  $R^2$  is isobutyl.

6. A process as defined in claim 1, wherein in said metal collector  $R^1$  is ethyl and  $R^2$  is pentyl.

7. A process as defined in claim 1, wherein said aqueous pulp slurry is provided by steel ball milling or autogenous or semi-autogenous milling the ore in water until liberation-sized ore particles are obtained.

8. A process as defined in claim 1, wherein said aqueous pulp slurry has a solids content of from about 10% to about 60%.

9. A process as defined in claim 1 wherein the pulp slurry is conditioned in step (b) by adding the frothing agent and metal collector to the pulp slurry under constant agitation and permitting agitation to continue until conditioning is substantially complete.

10. A process as recited in claim 9, wherein said conditioning step (b) is performed in a flotation cell.

11. A process for the beneficiation of base metal sulfide minerals from base metal sulfide ores with selective rejection of gangue sulfide minerals at a pH value of less than 7.0, said process comprising:

- (a) providing an aqueous pulp slurry of finely divided, liberation-sized ore particles having a solids content of from about 10% to about 60%;
- (b) adjusting the pH of said pulp slurry, if required, to below about 7.0, with sulfuric acid;
- (c) conditioning said pulp slurry with effective amounts of a frothing agent and a metal collector, respectively; said metal collector comprising at least one hydrocarboxycarbonyl thionocarbamate compound having the formula:



wherein  $R^1$  is  $C_1-C_6$  alkyl and  $R^2$  is  $C_1-C_8$  alkyl;

(d) thereafter, frothing the base metal sulfide minerals by froth flotation;

(e) and recovering the base metal sulfide materials.

12. A process as recited in claim 11, wherein the pH of the pulp slurry is adjusted to between 3.5 and 5.0 with sulfuric acid.

13. A process for beneficiation of bulk sulfides from complex sulfide ores, said process comprising:

- (a) providing an aqueous pulp slurry of finely divided, liberation-sized ore particles having a pH of between about 6.0 to 9.0, inclusive;
- (b) conditioning said pulp slurry with an effective amount of a frothing agent and from about 0.1 to about 1.0 lbs/ton of a metal collector, respectively, said metal collector comprising at least one hydrocarboxycarbonyl thionocarbamate compound having the formula:



wherein  $R^1$  is  $C_1-C_6$  alkyl and  $R^2$  is  $C_1-C_8$  alkyl;

(c) thereafter, frothing the bulk sulfide minerals by froth flotation;

(d) and recovering the base metal sulfide minerals.

\* \* \* \* \*